

March 7, 1967

K. STIEHL ET AL

3,307,961

METHOD OF PRODUCING AIR PERMEABLE SHEET MATERIAL

Filed Nov. 21, 1963



INVENTORS

KARL STIEHL  
KLAUS OEVERLÄNDER,

Reiley, Stephens & Huelting  
ATTORNEYS

3,307,961

## METHOD OF PRODUCING AIR PERMEABLE SHEET MATERIAL

Karl Stiehl and Klaus Oberländer, Hanau am Main, Germany, assignors to Deutsche Gold- und Silber-Scheideanstalt vormals Roessler, Frankfurt am Main, Germany

Filed Nov. 21, 1963, Ser. No. 325,433

Claims priority, application Germany, Nov. 21, 1962,

D 25,864

6 Claims. (Cl. 117—4)

The present invention relates to an improved process for the production of air permeable sheet materials especially suitable as upholstery, coverings, linings and the like.

The usual synthetic leather types, coated or lacquered textile fabrics, such as woven fabrics, knitted fabrics or fleeces, as well as foils which have been used for upholstery, coverings or linings are neither air permeable nor permeable to water vapor. In order to prepare air permeable material for the applications indicated it is known, for example, that the synthetic leather or similar materials can be perforated subsequent to their production. It is furthermore known that pierced synthetic leather like material can be produced in that the moving carrier web during application of an elastic synthetic resin layer is perforated by a heated roller which in addition to being provided with engraving depressions is provided with a large number of engraving points. However, both methods have not achieved wide acceptance. It is especially disadvantageous that the textile carrier is damaged during the perforating or piercing operation. In addition, the opposing roll, despite the use of special embossing rollers, is subject to strong wear. Furthermore, the limited selection of designs is also of disadvantage. In addition, the perforations give the products an unpleasant noticeably artificial appearance. In addition, when embossing and perforation are carried out as separate operations, it is impossible or very difficult to orient the perforations and the embossed design with respect to each other, especially when complicated designs are concerned.

A process furthermore is known in which the coating on the fabric is pressed aside all the way down to such fabric in individual locations with the aid of especially deep stampings in order to attain a certain porosity. The air permeability thus attained, especially with heavier qualities is only slight and in addition the bond and, under some circumstances, also the fabric are damaged.

The object of the present invention is to provide a simple and inexpensive process for the production of a tear-resistant, flexible, weldable, perforated sheet material which is especially adapted as upholstery, coverings, linings, decoration and the like. The sheet material according to the invention consists essentially of an open or wide meshed fiber structure as a base which is coated on one or both sides with a thermoplastic synthetic resin having spaced openings therein produced by stamping the synthetic resin coating so deeply that at least one side is provided with spaced hollow nob like protrusions and then grinding or cutting off such protrusions.

In the production of the coated sheet materials according to the invention, care should be taken that the fabric base is sufficiently open meshed, that is, that a sufficient space is provided between the individual threads of, for example, one to several millimeters. The fabric can, for example, be of basket weave or netting weave with twist bond. With usual thread strengths of about 20 to 3000 denier, preferably about 1000 to 2000 denier, a warp and woof density of about 2 to 12 threads per centimeter, preferably about 5 threads per centimeter, should be em-

ployed. The threads preferably are multifilament threads and preferably are of synthetic fibers, such as, for example, of regenerated cellulose, polyamides, polyesters, such as polyethylene glycol terephthalate, polyacrylonitrile, polycarbonates, or their copolymers, or other polymers customarily employed for the production of fibers. Fibers of natural origin can also be employed for the fabric base. In addition to woven fabrics, knitted fabrics, or fabric fleeces, which also must be of similar wide meshed or open nature, can be employed as the fiber structure serving as the base for the thermoplastic resin coating or covering. The especially important advantage of such open fiber structures is that only a few if any fibers are damaged during the deep stamping operation, so that practically no weakening of the fabric base results. Furthermore, the synthetic resin coating applied to such base increases the strength of the end product without unduly reducing the flexibility of the end product.

The stamping of the synthetic resin can be effected to produce the nob like protrusions on both sides of the sheet material but preferably on only one side thereof. According to the invention the deep stamping is effected simultaneously with the normal decorative graining or embossing operation with the aid of a suitably contoured embossing roll. Therefore the embossing roll in addition being provided with the usual embossing design is also provided with spaced relatively long spurs and/or relatively deep depressions corresponding in number and shape to the openings which are to be achieved. The length of such spurs or depressions with reference to the usual embossing design being such that when a resilient opposing roll is employed hollow nob like protrusions are respectively either effected in the sheet material on the side opposite to the decorative design or the same side as the decorative design. Such spurs can have any type of cross-section, but preferably are round, oval, angular or star-shaped and press the resin coated fabric through sufficiently far that nob like projections are provided, preferably on the reverse side from the side of the decorative embossed design, which projections can then be ground or cut off without difficulty, for example, in a subsequent operation with the aid of knife-, shearing- or grinding rolls.

The roll opposing the embossing roll preferably is a rubber roll of not too great a hardness, for example, of a Shore hardness of 60-70°.

If the back side of the sheet material is also coated with thermoplastic synthetic resin, such back side can also be embossed after embossing the front side and cutting off the projections produced on such back side during the first embossing operation.

The embossing of the sheet material according to the invention preferably is carried out at temperatures within the thermoplastic range of the resin employed for the coating. Instead of employing the embossing rolls which are preferably employed according to the invention, it is also possible to carry out the embossing discontinuously, using embossing stamps.

All known thermoplastic resins or resin mixtures, especially, those containing plasticizers, suitable for the production of coatings and foils can be employed as the coating material according to the invention. Coating masses based on plastisols of polyvinyl halides, such as those produced from vinyl chloride or vinylidene chloride or mixtures thereof, have proved particularly suited, as they permit the production of a material which is especially adapted to be welded.

The sheet materials produced according to the invention are especially adapted for upholstery, covering, decorations, linings and the like, particularly for the automotive industry. They combine good appearance, which can be improved with the use of colored or vari-colored

resin coatings, with very good strength and mechanical resistance. The air permeability is very good while permitting hard wear. The type and density of the perforations employed permit wide variations in air permeability. The air permeability is of special advantage when such material is employed as upholstery material. The sheet material according to the invention can, however, be employed with advantage in the production of shoes and luggage. Again in such applications the good appearance of the sheet material is of special advantage, particularly when the perforations fit in well with the embossed design which was produced in the same operation as provided for the location and shape of the perforations ultimately obtained in such material.

eter diagonally spaced 6 mm. apart on the coated side against an opposing rubber roll of a Shore hardness of 60-70°. The embossing was carried out at a temperature within the thermoplastic range of the plasticized polyvinyl composition. After the embossed fabric cooled down the hollow nob like protrusions caused by the spurs on the embossing roll were sheared off to leave spaced perforations (about 350 per dm.<sup>2</sup>) about 1.5 mm. in diameter in the finished embossed sheet.

The material produced had the mechanical properties indicated in the following table in which K signifies in the direction of the warp and S signifies in the direction of the woof.

TABLE

| Tensile Strength,<br>kg./5 cm. |    | Elongation on<br>break in percent |    | Resistance to<br>Tear Propagation<br>(according to<br>DIN 53356) |    | Air Permeability,<br>liters/minute/100<br>cm. <sup>2</sup> at 20 mm.<br>water column<br>pressure |
|--------------------------------|----|-----------------------------------|----|------------------------------------------------------------------|----|--------------------------------------------------------------------------------------------------|
| K                              | S  | K                                 | S  | K                                                                | S  |                                                                                                  |
| 65                             | 68 | 24                                | 26 | 18                                                               | 17 | 360                                                                                              |

The material can be processed by all of the customary procedures, such as, adhesive bonding, sewing or welding. Of special importance is its capability of being welded together, not only with itself but also other synthetic leathers or foils and even with ordinary textile upholstery materials, preferably with the aid of high frequency heating.

In the accompanying drawing:

FIG. 1 diagrammatically discloses an apparatus suitable for carrying out the process according to the invention; and

FIG. 2 shows a top plan view of a sheet material produced according to the invention having the openings produced therein oriented with respect to the embossed design.

Referring to the drawing, a web 1 of open meshed netting is passed through coating tank 2 and the resulting coated web 3 is passed through a heated gelling chamber 4. The heated gelled coated fabric is passed through an embossing calender composed of embossing roll 5 provided with engraved design depressions 6 with spaced spurs 6' and opposing rubber roll 7. The embossed coated fabric which now has been provided with hollow nob like projections 8 caused by spurs 6' after cooling is passed through cutter 9 whereby the nob like projections are cut off, leaving perforations 10 in the coated fabric.

The following example will serve to illustrate the invention.

#### Example

A polyester (polyethylene glycol terephthalate) woven netting having a thread count of 5 multifilament threads of 1000 denier in both warp and woof was placed over a polyvinyl chloride sheet 0.2 mm. thick which had been produced from a plastisol of the following composition:

| Percent by weight                                                 |      |
|-------------------------------------------------------------------|------|
| Polyvinyl chloride (emulsion polymer of a K value<br>of about 75) | 50   |
| Diocetylphthalate                                                 | 40   |
| Paraffin                                                          | 0.31 |
| Pigment and filler (titanium dioxide)                             | 8.94 |
| Dibutyl tin maleate                                               | 0.75 |

Thereafter the upper side of the associated netting and sheet was coated twice with a plastisol of the same composition so as to apply a total coating of 300-400 g./m.<sup>2</sup>. The composite structure was then heated and calendered.

Subsequently the material was embossed with an embossing roll provided with spurs about 1.5 mm. in diam-

The thickness of such product was 1.1 mm. and its weight was 850 g./m.<sup>2</sup>.

The use of the open meshed fabric base instead of a close meshed fabric was in part responsible for the lessened damage to such fabric in the production of the perforated product. On the other hand, the spurs on the embossing rolls in producing the nob like projections which were later sheared off tended to displace the threads of the fabric base laterally rather than damage them whenever such threads happened to be in the path of such spurs.

We claim:

1. A method of producing air permeable thermoplastic sheet material reenforced with a fiber fabric which comprises coating at least one side of an open meshed fiber fabric with a continuous coating of a thermoplastic synthetic resin, embossing such coating at a temperature within the thermoplastic range thereof with a decorative design while simultaneously in the same operation embossing such coating so deeply as to provide spaced hollow nob like protrusions from at least one side thereof and removing such nob like protrusions to provide spaced openings in such sheet material.

2. The method of claim 1 in which said open meshed fabric has a thread count in both warp and woof of about 2 to 12 threads per centimeter, the thread size being between 20 and 3000 denier.

3. The method of claim 1 in which said open meshed fabric has a thread count in both warp and woof of about 5 threads per centimeter, the thread size being between 1000 and 2000 denier.

4. The process of claim 1 in which the nob like protrusions caused by the deep embossing protrude from the side of the sheet material opposite to that receiving the embossed decorative design.

5. The process of claim 4 in which said protrusions and the openings resulting therefrom are oriented with respect to the decorative design.

6. The process of claim 1 in which said coating is of plasticized polyvinyl chloride.

#### References Cited by the Examiner

#### UNITED STATES PATENTS

|    |           |         |         |          |
|----|-----------|---------|---------|----------|
| 70 | 2,817,596 | 12/1957 | Schur   | 117-4    |
|    | 2,861,006 | 11/1958 | Salditt | 117-11 X |
|    | 3,137,893 | 6/1964  | Gelpke  | 117-4 X  |
|    | 3,214,502 | 10/1965 | Schaar  | 117-4 X  |